

## UNITED STATES PATENT OFFICE

2,188,900

LIGHT SENSITIVE PAPER AND SENSITIZING  
COMPOSITION THEREFORGustav A. Hinkel, Pittsburgh, Pa., assignor to  
B. K. Elliott Company, Pittsburgh, Pa., a cor-  
poration of PennsylvaniaNo Drawing. Application February 20, 1939,  
Serial No. 257,331

## 24 Claims.

## (Cl. 95—6)

My invention relates to the art of preparing light sensitive papers, cloth and other suitable materials, hereinafter referred to generally as "paper" and in their sensitized form as "blue print paper", for use in making reproductions, especially of plans and line work by superimposing upon the blue print paper a drawing, tracing or the like made on transparent or translucent material, exposing it to the light and then developing it by means of successive treatments with water and an oxidizing agent.

The principal object of my invention is the provision of a sensitized composition for the production of an improved blue print paper of exceedingly fine keeping qualities, unusually high printing speed and minimized tendency to curl.

Prints made from my improved paper show great contrasts due to very dark blue backgrounds and decidedly pure white details. Furthermore these prints are extremely resistant to the bleaching effect of the light rendering them practically fade proof.

As is known to those skilled in the art, blue print papers are commonly prepared by coating a suitable paper with a sensitizing composition consisting of an aqueous solution of ferric alkali metal salts of organic acids, such as ferric ammonium oxalate, and an alkali metal ferricyanide such as potassium ferricyanide. Due to the gradual, spontaneous change of the alkali metal ferricyanide into an alkali metal ferrocyanide, for example potassium ferrocyanide, and its subsequent interaction with the ferric ammonium oxalate simultaneously present in the light sensitive layer, a blue compound commonly termed "Prussian blue" is formed prior to exposure to the light. This compound will be referred to hereinafter as "Prussian blue" irrespective of the scientific correctness of its name.

This Prussian blue is insoluble in the water which is used for washing the prints in the process of their development, causing the lines and other details of the blue prints to assume a bluish tinted appearance. Since this tinting materially decreases the contrasts in these prints, blue print papers coated with that type of sensitizing composition are unsatisfactory.

Satisfactory results as to producing white details are known to be obtainable by the addition of an acid, such as phosphoric acid or oxalic acid, or an acid alkali metal salt such as sodium binoxalate or ammonium dihydrogen phosphate, or a alkaline hydrolyzing alkali metal salts such as sodium oxalate or potassium monohydrogen phosphate, to the sensitizing compositions comprising an aqueous solution of, for example, ferric ammonium oxalate and potassium ferricyanide. Owing to their capability of changing

soluble compound more or less white lines or details are characteristic of prints made from paper coated with a sensitizing composition containing a certain amount of aforementioned acids, acid salts or alkaline hydrolyzing salts, besides ferric alkali metal salts of organic acids and alkali metal ferricyanides. Despite the obvious advantage of improved contrasts and undisputed superior keeping qualities of these blue print papers they, nevertheless, lack a satisfactory printing speed.

More recently and as disclosed in British Patent No. 418,369 to J. Halden & Company, Limited, and United States Patent No. 2,093,738 to Alger P. Reynolds, alkali metal ferrocyanides, such as potassium ferrocyanide, sodium ferrocyanide or ammonium ferrocyanide, are used as the full or partial substitute for alkali metal ferricyanides, such as potassium ferricyanide, sodium ferricyanide or ammonium ferricyanide contained in heretofore employed blue print paper sensitizing solutions. The purpose of this is to eliminate or minimize the obviously light screening action of the traditionally used, strongly yellow colored alkali metal ferricyanides.

Under ordinary circumstances the presence of alkali metal ferricyanides in blue print paper sensitizing solutions containing organo alkali metal ferric salts, such as ferric ammonium oxalate, and alkali metal ferricyanides such as potassium ferricyanide, would as stated supra cause the formation of Prussian blue, and paper coated with such a solution would be unsatisfactory, despite its faster printing speed, due to the fact that blue prints made from this paper show strongly blue colored lines instead of contrasting white lines on a blue background. Therefore the presence of Prussian blue, even though finely suspended, renders the composition unsuitable as a sensitizing solution for blue print paper.

Both the above mentioned patents call for the addition to this sensitizing solution of certain ingredients to prevent the formation of Prussian blue. These are referred to as alkaline buffer salts of alkali metals or alkaline hydrolyzable alkali metal compounds. According to both patent disclosures the ingredients used to make up this type of blue print sensitizing solution, which hereinafter will be referred to as "ferrocyanide blue print solution", are similar if not identical and so are the solutions, with the exception of the final acidity or more correctly the value of the hydrogen ion concentration or, in other words, the pH value of both types of solution; Holden's ferrocyanide blue print solution being neutral or slightly alkaline claiming a pH value of 7 or higher while Reynolds' solution is acid claiming a pH value of lower than 7.

I discovered a new and useful method of preventing the formation of Prussian blue in ferro-

cyanide blue print solutions by means of incorporating into such compositions salts consisting of a dibasic or tribasic acid either organic or inorganic and a hydroxyalkyl amine either a primary, secondary or tertiary amine irrespective of the final pH value of such solutions, although I prefer a pH value of 7 or below 7 but preferably not below 3.

The particular advantage of using hydroxyalkyl amine salts lies in their comparatively great solubility in water which, for example, in the case of tri hydroxyethyl amine oxalate is unlimited. This fact and the fact that hydroxyalkyl amines readily dissolved basic ferrous salts of organic acids, assumed by the art to be present in the background of the prints after exposure to the light, provides for speedy development into blue prints of unexcelled fastness to light and which may be more fully explained by the following facts:

The process of development consists mainly in washing the prints with water thereby removing all the chemicals that are not affected or are only partially affected by the actinic rays of the light thus fixing the white lines or details of the print, and removing all the chemicals which have no part in the formation of the blue background of the print, especially the abovementioned basic ferrous salts of organic acids. The process further comprises the oxidation of the originally light colored background into a deep blue. It is to be noted that the incomplete removal of the basic ferrous salts results in their subsequent oxidation into light sensitive ferric salt and this in turn is the reason for bleaching when those prints are exposed to the light.

Another advantage of using hydroxyalkyl amine salts and particularly tri hydroxyethyl amine oxalate lies in their slight hygroscopicity which is less than for instance that of glycerin but high enough to act as a humidifying agent for the paper, thus producing in the sensitized material a higher grade of suppleness. This action on the paper is facilitated owing to the fact that a number of hydroxyalkyl amine salts, such as di hydroxyethyl amine oxalate, tri hydroxyethyl amine phosphate, tri hydroxyisopropyl amine oxalate, and others known to those skilled in the art, are at commonly prevailing temperatures of a viscous oily consistency, instead of being solid crystals as is the case with alkali metal salts. This improved suppleness is especially desirable in sheetprinting where stiff sheets of blue print paper having a tendency to curl and to roll up retard production.

Among the salts capable of preventing the formation of undesirable Prussian blue in ferrocyanide blue print solutions and falling within the scope of this invention, without limiting myself thereto, are the following: mono hydroxymethyl amine oxalate, mono hydroxyethyl amine phosphate, mono hydroxyethyl amine citrate, mono hydroxypropyl amine tartrate, mono hydroxyisopropyl amine oxalate, di hydroxyisopropyl amine oxalate, di hydroxyethyl amine oxalate, di hydroxyisobutyl amine phosphate, tri hydroxyethyl amine tartrate, tri hydroxyethyl amine oxalate, tri hydroxymethyl amine phosphate, tri hydroxypropyl amine tartrate, tri hydroxyisopropyl amine borocitrate, tri hydroxybutyl amine glycerophosphate and others known to those skilled in the art.

Within the scope of the discovery are complex salts consisting of a residue of a suitable dibasic acid and a suitable metal of the first or second

group of the periodical arrangement of the element not forming water insoluble compounds with ferrocyanide or ferricyanide ions and either primary, secondary or tertiary hydroxyalkyl amines. By "suitable dibasic" acid I mean such acids as tartaric acid, oxalic acid, malic acid and others known to the ones skilled in the art. By "a suitable metal of the first or second group" in the above connection, I am referring to such metals as sodium, potassium, ammonium which although not strictly a metal is generally classed here, magnesium, calcium and others known to the ones skilled in the art. Complex salts of the type which I am referring to are such as tri hydroxyethyl amine potassium oxalate, di hydroxyisopropyl amine sodium tartrate, tri hydroxymethyl amine ammonium malate and others known to those skilled in the art.

I also include complex salts consisting of a suitable tribasic acid such as phosphoric acid, citric acid, boric acid, and one or two suitable metals of the first or second group of the periodical arrangement of the elements which do not form water insoluble compounds with ferrocyanide or ferricyanide ions which are referred to in the preceding paragraph, and one or two, as the case may be, of the mono, di, or tri hydroxyalkyl amines, particularly salts such as mono di hydroxyethyl amine sodium hydrogen phosphate, mono tri hydroxyisopropyl sodium magnesium citrate, mono hydroxymethyl potassium glycerophosphate and similar salts known to those skilled in the art.

I furthermore include complex salts of a di or tribasic acid, such as mentioned above, and two or three, as the case may be, different mono, di or tri hydroxy alkyl amines. Salts in this class are as follows: Di hydroxyethyl amine tri hydroxy methyl amine oxalate, tri hydroxyisopropyl amine tri hydroxyethyl amine hydrogen phosphate, mono hydroxyethyl tri hydroxyethyl tri hydroxypropyl amine citrate and other similar salts known to those skilled in the art.

It is within the scope of this invention to use any such acids and bases or acid and alkaline reacting chemicals which when added to the ferrocyanide blue print solution would give rise to the formation of salts or complex salts of the aforescribed nature.

The following examples are ferrocyanide blue print solutions typical for this invention:

#### Example #1

|                                |        |       |
|--------------------------------|--------|-------|
| Water                          | ccs.   | 1,000 |
| Tri hydroxyethyl amine oxalate | grams. | 150   |
| Sodium ferro-cyanide           | do     | 40    |
| Potassium ferricyanide         | do     | 10    |
| Ferric ammonium oxalate        | do     | 150   |

the amount of tri hydroxyethyl amine oxalate being used as a restrainer to prevent the formation of Prussian blue can be varied and if so should be regulated in accordance with the amount of sodium ferrocyanide substituting for potassium ferricyanide. If more hydroxyalkyl amine salt is used than is required to prevent the forming of Prussian blue, then the printing speed of the paper coated with such a solution will be retarded although its keeping qualities are improved without the rich blue color of the background and the clear white of the details being affected disadvantageously. If the amount of potassium ferricyanide is increased without changing the other ingredients of above formula, the blue background will be deepened, but at the expense of the reduction of the printing speed. The keeping qualities as well as the whiteness

of the details are not only retained but rather improved.

In Example #1 tri hydroxyethyl amine oxalate is being used as a restrainer to prevent the formation of Prussian blue. Equivalent amounts of 5 tertiary hydroxyalkyl amine oxalates other than tri hydroxyethyl amine oxalate, can be substituted therefor, such salts as tri hydroxymethyl amine oxalate, tri hydroxyisopropyl amine oxalate, tri hydroxybutyl amine oxalate and similar ones. Equivalent amounts of primary and secondary hydroxyalkyl amine oxalates can also take the place of tri hydroxyethyl amine oxalate, and I name salts such as mono hydroxymethyl 10 amine oxalate, mono hydroxyethyl amine oxalate, mono hydroxybutyl amine oxalate, di hydroxyethyl amine oxalate, di hydroxypropyl amine oxalate, di hydroxyisobutyl amine oxalate and others known to those skilled in the art. I 15 note that the acid residues of di and tri basic acids such as tartaric acid, malic acid, boric acid, phosphoric acid, glycerophosphoric acid and others known to those skilled in the art can take the place of the residue of oxalic acid of the 20 tri hydroxyethyl amine oxalate used in the formula of Example #1.

Another example of a suitable sensitizing solution is as follows:

*Example #2*

|                                         |       |       |
|-----------------------------------------|-------|-------|
| 30 Water                                | ccs   | 1,000 |
| Di hydroxyethyl amine potassium oxalate | grams | 120   |
| Sodium ferrocyanide                     | do    | 35    |
| 35 Potassium ferricyanide               | do    | 15    |
| Ferric ammonium oxalate                 | do    | 150   |

In this ferrocyanide blue print solution a complex salt is used as a restrainer to prevent formation of Prussian blue. It consists besides 40 the oxalic acid residue of the alkali metal potassium and the secondary hydroxyalkyl amine di hydroxyethyl amine. In this formula, too, any other suitable primary, secondary or tertiary hydroxyalkyl amine may take the place of above 45 mentioned secondary amine, and any other suitable metal of the first or second group of the periodically arranged system of the elements may be substituted for potassium such as sodium, lithium, ammonium (this latter one although 50 not strictly a metal is generally classed here), magnesium, strontium and others known to those skilled in the art. The alkali metal potassium can furthermore be replaced by any such primary, secondary and tertiary hydroxyalkyl amines as 55 hereinbefore mentioned.

Instead of the residue of oxalic acid other such acid residues as already referred to under Example #1 can form the acid constituent of complex salts intended to be used in the formula of 60 Example #2.

Another formula for a suitable ferrocyanide solution is given as follows:

*Example #3*

|                            |       |       |
|----------------------------|-------|-------|
| 65 Water                   | ccs   | 1,000 |
| Oxalic acid                | grams | 37.8  |
| Tri hydroxyethyl amine     | do    | 89.4  |
| Sodium ferrocyanide        | do    | 30    |
| Potassium ferricyanide     | do    | 20    |
| 70 Ferric ammonium oxalate | do    | 165   |

This ferrocyanide blue print solution is similar as to its characteristics to the one given as Example #1. Although the two ingredients oxalic acid and tri hydroxyethyl amine are not recorded in that formula the similarity of both 75

solutions is established through the fact that the stoichiometrically equivalent amounts of oxalic acid and tri hydroxyethyl amine which are used in Example #3 form tri hydroxyethyl amine oxalate when dissolved. It is understood that in this formula the hydroxyalkyl amine base need not necessarily be tri hydroxyethyl amine. Equivalent amounts of any other suitable primary, secondary and tertiary hydroxyalkyl amine base together with stoichiometrically equivalent 10 amounts of other suitable dibasic or tribasic acids other than oxalic acid and known to those skilled in the art can take its place.

It is within the scope of this invention to use various suitable acids simultaneously with either 15 one or any number of corresponding amounts of hydroxyalkyl amine bases to form mixtures of hydroxyalkyl amine salts.

Another formula for a suitable ferrocyanide blue print solution is given as follows:

*Example #4*

|                            |       |       |
|----------------------------|-------|-------|
| Water                      | ccs   | 1,000 |
| Tri hydroxyisopropyl amine | grams | 59.4  |
| Potassium binoxalate       | do    | 46.2  |
| Sodium ferrocyanide        | do    | 25    |
| Potassium ferricyanide     | do    | 25    |
| Ferric ammonium oxalate    | do    | 150   |

The ferrocyanide blue print solution made up according to this formula is similar as to the 30 characteristics of its ingredients to Example #2, inasmuch as the stoichiometrically equivalent amounts of potassium binoxalate and tri isopropyl amine form a complex salt, i. e. tri hydroxyisopropyl amine potassium oxalate when dissolved together in the required amount of water. I do not intend to limit myself to the use of 35 potassium binoxalate as the only acid salt, nor to the use of tri hydroxyisopropyl amine as the only hydroxyalkyl amine base forming complex 40 salts used as restrainers to prevent formation of Prussian blue in ferrocyanide blue print solutions. I include any other suitable acid salts such as the binoxalates, the bitartrates, the bimalates, the mono hydrogen phosphates and citrates, the di hydrogen phosphates and citrates of the metals of first and second group of the 45 periodically arranged system of the elements including ammonium and also including any of the primary, secondary and tertiary hydroxyalkyl amine bases hereintofore mentioned such as the binoxalates of ammonium, sodium magnesium, hydroxyalkyl amine bases, the bitartrates of potassium, sodium, ammonium and hydroxyalkyl amine bases, the mono hydrogen 50 phosphates of potassium, sodium, ammonium magnesium and hydroxyalkyl amines and many others known to those skilled in the art.

Instead of tri hydroxyisopropyl amine any other hydroxyalkyl amine base such as mentioned in the explanatory paragraphs following 55 Example #3 are suitable to be used.

Another formula for a suitable ferrocyanide blue print solution is given as follows:

*Example #5*

|                            |       |       |
|----------------------------|-------|-------|
| Water                      | ccs   | 1,000 |
| Oxalic acid                | grams | 18.6  |
| Potassium oxalate          | do    | 27.2  |
| Tri hydroxyethyl amine     | do    | 44    |
| Sodium ferrocyanide        | do    | 20    |
| Potassium ferricyanide     | do    | 25    |
| 70 Ferric ammonium oxalate | do    | 160   |

The stoichiometrically equivalent amounts of 75 oxalic acid, potassium oxalate and tri hydroxy-

ethyl amine mentioned above form when brought in solution tri hydroxyethyl amine potassium oxalate. Thus this ferrocyanide solution is in every respect similar to the solutions prepared 5 in accordance with the formulae of Examples #2 and #4, all three solutions containing complex salts after solution has been effected. It is unnecessary to enumerate all the possibilities as to suitable acids that can be used instead of 10 oxalic acid neither need I mention the various salts of di and tri basic acids to substitute for potassium oxalate or other hydroxyalkyl amines to take the place of tri hydroxyethyl amine, these being evident, to those skilled in the 15 art, from the foregoing paragraphs.

It is understood that the amounts of ingredients in any of the referred to examples are not given with the intention of confining myself strictly to these figures or ratios or multiples 20 of them any one of these amounts being subject to changes. Neither do I intend to restrict the number of ingredients of my new type of ferrocyanide blue print solution to the number of ingredients recorded in those examples. I prefer for instance to add small amounts of from 1 to 5 grams of an acid such as oxalic acid, citric acid, tartaric acid, phosphoric acid to herein-referred to formulae with the purpose of accelerating the printing speed of the paper coated 25 with said solutions. I furthermore include additions such as saponine or sulphonated fatty acids to facilitate their absorption by particularly hard papers and catalysts such as salts of vanadic acid to increase the printing speed of this new 30 type of blue print paper. I am aware of the fact that ferric ammonium oxalate used in all examples as the light sensitive ferric alkali metal salt is a complex salt and can be replaced by any other organo ferric salt together with alkali 35 metal salts of di or tri basic organic acids to form complex salts when dissolved.

I claim:

1. A sensitizing composition for blue print paper and the like which comprises an aqueous solution of a ferric alkali metal salt of an organic acid, an alkali metal ferrocyanide, and a hydroxyalkyl amine salt of a polybasic acid.

2. A sensitizing composition for blue print paper and the like which comprises an aqueous 50 solution of a ferric alkali metal salt of an organic acid, an alkali metal ferrocyanide, an alkali metal ferricyanide, and a hydroxyalkyl amine salt of a polybasic acid.

3. A sensitizing composition for blue print paper and the like comprising an aqueous solution in accordance with claim 1, wherein the hydroxyalkyl amine salt is tri hydroxyethyl amine oxalate.

4. A sensitizing composition for blue print paper and the like comprising an aqueous solution in accordance with claim 2, wherein the hydroxyalkyl amine salt is tri hydroxyethyl amine oxalate.

5. A sensitizing composition for blue print paper and the like which comprises an aqueous solution of a ferric alkali metal salt of an organic acid, an alkali metal ferrocyanide, and a complex salt of a polybasic acid with a hydroxyalkyl amine base, and a suitable metal of the 65 first or second group of the periodically arranged system of the elements.

6. A sensitizing composition for blue print paper and the like which comprises an aqueous solution of a ferric alkali metal salt of an organic acid, an alkali metal ferrocyanide, an alkali metal

ferricyanide, and a complex salt of a polybasic acid with a hydroxyalkyl amine base, and a suitable metal of the first or second group of the periodically arranged system of the elements.

7. A sensitizing composition for blue print 5 papers and the like comprising an aqueous solution in accordance with claim 5, wherein the complex salt is tri hydroxyethyl amine potassium oxalate.

8. A sensitizing composition for the print 10 papers and the like comprising an aqueous solution in accordance with claim 6, wherein the complex salt is tri hydroxyethyl amine potassium oxalate.

9. Blue print paper and the like having a 15 light-sensitive coating comprising a ferric alkali metal salt of an organic acid, an alkali metal ferrocyanide and a hydroxyalkyl amine salt of a polybasic acid.

10. Blue print paper and the like having a 20 light-sensitive coating comprising a ferric alkali metal salt of an organic acid, an alkali metal ferrocyanide, an alkali metal ferricyanide, and a hydroxyalkyl amine salt of a polybasic acid.

11. Blue print paper and the like having a 25 light-sensitive coating of the character in accordance with claim 9, wherein the hydroxyalkyl amine salt is tri hydroxyethyl oxalate.

12. Blue print paper and the like having a 30 light-sensitive coating of the character in accordance with claim 10, wherein the hydroxyalkyl amine salt is tri hydroxyethyl oxalate.

13. Blue print paper and the like having a 35 light-sensitive coating comprising a ferric alkali metal salt of an organic acid, an alkali metal ferrocyanide, and a complex salt of a polybasic acid with a hydroxyalkyl amine base, and a suitable metal of the first or second group of the periodically arranged system of the elements.

14. Blue print paper and the like having a 40 light-sensitive coating comprising a ferric alkali metal salt of an organic acid, an alkali metal ferrocyanide, an alkali metal ferricyanide, and a complex salt of a polybasic acid with a hydroxyalkyl base, and a suitable metal of the first or 45 second group of the periodically arranged system of the elements.

15. Blue print paper and the like having a 50 light-sensitive coating of the character in accordance with claim 13, wherein the hydroxyalkyl amine salt is tri hydroxyethyl oxalate.

16. Blue print paper and the like having a 55 light-sensitive coating of the character in accordance with claim 14, wherein the hydroxyalkyl amine salt is tri hydroxyethyl oxalate.

17. A product consisting of an adaptable base and a light-sensitive layer thereon containing a ferric alkali metal salt of an organic acid, an alkali metal ferrocyanide, and a hydroxyalkyl amine salt of the 60 polybasic acid.

18. A product consisting of an adaptable base and a light-sensitive layer thereon containing a ferric alkali metal salt of an organic acid, an alkali metal ferrocyanide, an alkali metal ferricyanide, and a hydroxyalkyl amine salt of a polybasic acid.

19. A product in accordance with claim 17, wherein the hydroxyalkyl amine salt is tri hydroxyethyl amine oxalate.

20. A product in accordance with claim 18, 70 wherein the hydroxyalkyl amine salt is tri hydroxyethyl amine oxalate.

21. A product consisting of an adaptable base and a light-sensitive layer thereon containing a ferric alkali metal salt of an organic acid, an

alkali metal ferrocyanide, a complex salt of a polybasic acid with a hydroxyalkyl amine base, and a suitable metal of the first or second group of the periodically arranged system of the elements.

22. A product in accordance with claim 21 wherein the hydroxyalkyl amine salt is tri hydroxyethyl amine oxalate.

23. A product in accordance with claim 22 wherein the hydroxyalkyl amine salt is tri hydroxyethyl amine oxalate.

GUSTAV A. HINKEL. 10